

S. E. FORD.

## MANUFACTURE OF VARNISH.

APPLICATION FILED APR. 4, 1913.

1,109,979.

Patented Sept. 8, 1914.



**Witnesses:**

WITNESSES.  
Benjamin B. Hovey  
Green Arbor

Inventor:  
Stanley E. Ford,  
by Alfred J. Davis,  
His Attorney.

# UNITED STATES PATENT OFFICE.

STANLEY E. FORD, OF SCOTIA, NEW YORK, ASSIGNOR TO GENERAL ELECTRIC COMPANY, A CORPORATION OF NEW YORK.

## MANUFACTURE OF VARNISH.

1,109,979.

Specification of Letters Patent.

Patented Sept. 8, 1914.

Application filed April 4, 1913. Serial No. 758,832.

To all whom it may concern:

Be it known that I, STANLEY E. Ford, a citizen of the United States, residing at Scotia, in the county of Schenectady, State 5 of New York, have invented certain new and useful Improvements in the Manufacture of Varnish, of which the following is a specification.

My invention relates to the manufacture 10 of varnish, one of the objects of my invention being to reduce the cost of making the varnish by reducing the amount of time required for the operation.

In the varnish-making processes as usually employed the varnish materials are boiled in open kettles for a long period, generally twenty-four hours or more. This slow process naturally increases the cost of the varnish.

20 In one embodiment of my invention the varnish-forming liquid is reduced to a finely divided form so as to bring an oxidizing atmosphere such as ozone into intimate contact with the whole body of liquid 25 and thereby cause rapid oxidation. The varnish materials are preferably placed in a drum in which there is some agitating means, such as a paddle wheel, so arranged as to cause the liquid to be thoroughly subdivided and the ozone is introduced into the drum and acts upon the material in this form, the whole body of liquid being subjected to heat.

30 In the accompanying drawing I have illustrated a machine suitable for carrying out my invention.

In the drawing, Figure 1 is a side elevation partly in section of my machine and Fig. 2 is a sectional view of the same.

40 Referring to the drawing, 10 is a casing, preferably of metal, in the form of a cylinder or drum having supporting feet 11. This drum is provided with heads 12 and 13 secured to the casing so as to form a completely inclosed chamber. Within this chamber is a rotatable member 14 shown in the form of a paddle wheel having four vanes. I have shown the vanes as tapering both ways from the center so as to give the 45 liquid a tendency to collect toward the middle of the machine instead of piling up at the ends. This paddle wheel is mounted in the heads and is rotated by a pulley 15. The edges of the vanes are provided with

V-shaped scallops, as shown. These scallops 55 serve the purpose of increasing the linear dimensions of the edge of the vane and thereby increasing the length of the edge over which the liquid falls when it is carried to the top of the drum. This causes 60 the liquid to be reduced to a finely divided form so as to be in more intimate contact with the ozone. In fact, the materials may be so finely divided as to become a fine spray or froth which will render the action of the 65 ozone very effective. The drum may be heated in any desired manner, but I have shown for purposes of illustration an outer jacket 16 located on the lower portion of the drum through which steam is admitted 70 through the pipes 17. This heating jacket is surrounded by heat insulating lagging 18 held in place by the bands 19. The heat dispels any air pockets that may have a tendency to form in the liquid. Ozone is introduced into the chamber through the pipe 20 and the gaseous products are discharged into the air through pipe 21. The varnish materials are introduced through the hole 22 at the top and drawn off through a 80 spigot 23 at the bottom.

75 In making varnish in accordance with my invention the varnish materials are introduced through the hole 22 so as to about half fill the drum. Steam is turned into the 85 heating jacket so as to cause a temperature of from 300° to 450° F. within the drum. The paddle wheel 14 is then rotated rapidly, which causes the material to be carried to the top and toward the middle of the drum 90 in a fine spray upon which the ozone and heat act to cause rapid oxidation. I have found that six or seven hours suffices to produce an excellent grade of varnish by the use of this machine. This machine is 95 also used as a mixing tank, since after the oxidation is completed the solvent, which may be turpentine or gasoline, is added, nearly filling the drum, and by rotating the paddle wheel more slowly the materials are 100 thoroughly mixed and the varnish completed. It will be seen that the time used in the manufacture of varnish by my process is reduced to one-third or one-fourth of the time usually taken. Furthermore, the 105 process is practically automatic so that a single attendant can take care of a number of machines. The drums can be made much

larger than any kettle heretofore used. In fact, one of these drums may hold from fifty to one hundred barrels of varnish or more. All this, of course, goes to reduce the cost of the varnish and also makes the product more uniform. Furthermore, the loss of materials due to evaporation, which is a large factor in the making of varnish by the open kettle method, is greatly reduced.

10 Various modifications of my invention will suggest themselves to those skilled in the art without departing from the spirit of my invention, the scope of which is set forth in the annexed claim.

What I claim as new and desire to secure 15 by Letters Patent of the United States, is:—

The process of making varnish which consists in confining an oxidizable varnish forming liquid in a chamber under oxidizing conditions, applying heat to the liquid, 20 and agitating the same so as to reduce it to a fine spray.

In witness whereof, I have hereunto set my hand this 3rd day of April 1913.

STANLEY E. FORD.

Witnesses:

BENJAMIN B. HULL,  
HELEN ORFORD.